

## UNITED STATES PATENT OFFICE

2,524,725

## MAGENTA PHENAZONIUM DYESTUFF IMAGES FROM 8-HYDROXYQUINOLINE COUPLERS

Robert F. Coles, Easton, Pa., assignor to General Aniline &amp; Film Corporation, New York, N. Y., a corporation of Delaware

No Drawing. Application December 23, 1947,  
Serial No. 793,536

6 Claims. (Cl. 95—6)

1

The present invention relates to color formers of the 8-hydroxyquinoline class, which are particularly suitable for the production of magenta phenazonium dyestuff images by color development of an exposed silver halide emulsion with an orthophenylene diamine type color developer.

In the copending application Serial No. 640,382, filed on January 10, 1946, of Willy A. Schmidt and Vsevolod Tulagin, now Patent No. 2,486,440, there is described the production of phenazonium dyestuff images by color developing an exposed silver halide emulsion with a color developer comprising an ortho-phenylene diamine in the presence of a color former which may be inter alia 8-hydroxyquinoline.

It has now been discovered that the method of said application can be practiced to yield phenazonium dyestuff images having a markedly improved magenta transmission spectra by utilizing as the color formers 8-hydroxyquinolines (including 8-hydroxy cinchoninic acids) containing in the 2 position of the nucleus thereof an electronegative substituent such as a halogen or a mononuclear carbocyclic aromatic radical. It has been further found that such compounds readily lend themselves to the introduction of long alkyl chains to thereby render the color formers non-migratory in photographic emulsions, thus facilitating the employment of the color formers in photographic film. The photographic emulsions and color developers containing the aforementioned color formers and their use with orthophenylene diamine type developers to produce magenta phenazonium dyestuff images of improved spectral transmission constitute the purpose and objects of the present invention.

The 8-hydroxyquinolines, the use of which, as color formers, is contemplated herein, may be depicted by the following structural formula:



wherein R is an electronegative group such as a halogen, i. e., chlorine or bromine, or a mononuclear carbocyclic aromatic radical such as phenyl, nitro-phenyl, amino-phenyl, alkyl-sulfonamido-phenyl, alkyl-carboxamido-phenyl, in which if desired the alkyl radical may contain 10 or more carbon atoms, and the like, and R' represents hydrogen, carboxy, or a carboxamido group containing an alkyl chain of at least 10

2

carbon atoms, such as tetradecanoylamino, decanoylamino, dodecanoylamino, stearoylamino, and the like, or acylaminoaryl-carbamyl, such as stearoylamino - benzene - carbamyl, stearoylmethyl-sulfobenzene-carbamyl, and the like.

Examples of compounds embraced by the above formula are the following:

1.

10



2-chloro-8-hydroxyquinoline

15

2.



2-phenyl-8-hydroxy-cinchoninic acid

3.

20



2-(3-decylsulfonamidophenyl)-8-hydroxy cinchoninic acid

4.

25



2-(3-dodecylsulfonamidophenyl)-8-hydroxy cinchoninic acid

5.

30



2-bromo-8-hydroxy-quinoline

6.

35



2-(3-nitrophenyl)-8-hydroxy-quinoline

3



It will be apparent that in the compounds listed above, those containing an alkyl chain of at least 10 carbon atoms will be non-migratory in photographic emulsions. Consequently when these compounds are utilized, they must be dispersed in the photographic emulsions in order to be operable to produce the desired images on color forming development.

The color developers which are utilized are as stated of the ortho-phenylene diamine class, a large number of examples of which are referred to in the aforesaid Schmidt and Tulagin application. Suitable color developers are, for example: 4,6-dianilino metanilic acid, 4,6-bis-(o-methoxy-phenylamino) - metanilic acid, 4-(n-carboxy-phenylamino) - 6-(p-methoxy-phenylamino) - metanilic acid, 4,6-bis-(p-methoxy-phenylamino) -metanilic acid, and the like.

It is to be understood that the crux of the present invention is the color formers, and that any ortho-phenylene diamine type developer may be used with the color formers in producing the desired magenta phenazonium dye images.

The majority of the color formers previously referred to are known compounds. Those which are not described in the literature, such as that of Examples 3, 4, 8 and 11, can be prepared by the usual amidation reaction. For instance, the compound No. 3 may be obtained by reacting 2-

4

(3-aminophenyl)-8-hydroxy cinchoninic acid with decyl sulfonyl chloride in the presence of an acid-binding agent such as pyridine. A similar procedure is employed in producing the compound No. 4, the only difference being that lauryl sulfonyl chloride is used in forming the sulfonamide.

Compound No. 8 may be prepared by reacting 2-(3-amino-phenyl)-8-hydroxy cinchoninic acid with myristoyl chloride in the presence of an acid-binding agent such as pyridine.

Compound No. 10 may be formed by treating equimolecular proportions of 2-phenyl-8-hydroxy cinchoninic acid and octadecyl-taurine in pyridine solution with an excess of phosphorus trichloride dissolved in pyridine.

Compound No. 11 is formed by treating equimolecular proportions of 2-phenyl-8-hydroxy cinchoninic acid and 3-amino-6-stearoylaminotoluene-4-sulfonic acid in pyridine with an excess of phosphorus trichloride dissolved in pyridine.

The invention is illustrated by the following examples, but it is to be understood that these examples are illustrative and not limitative of the invention.

#### Example 1

A photographic silver bromide emulsion is exposed and then color developed for five to ten minutes in a solution of the following color developer:

|                              |       |      |
|------------------------------|-------|------|
| Sodium carbonate monohydrate | grams | 60   |
| Potassium bromide            | do    | 2.5  |
| Sodium sulfite               | do    | 40   |
| Pyridine                     | cc    | 12   |
| 4,6-dianilino metanilic acid | grams | 4    |
| 2-chloro-8-hydroxyquinoline  | do    | 2    |
| Water                        | cc    | 1000 |

40 The developed silver image is bleached with potassium ferricyanide and fixed in an acid hardening hypo solution. There is thus obtained a phenazonium dyestuff image which has a high magenta transmission spectrum.

45

#### Example 2

50 .5 gram of 2-(3-decylsulfonamidophenyl)-8-hydroxy cinchoninic acid is dissolved in 10 ml. of water by the addition of 1 N-sodium hydroxide solution. The solution of the color former is then added to 50 grams of a silver bromide emulsion and the emulsion coated on a film base.

55 The film after drying is exposed and developed with the developer of Example 1, excepting that the 2-chloro-8-hydroxyquinoline is omitted from the developing solution.

After working up the film as in Example 1, there is obtained a brilliant magenta dyestuff image having a high spectral transmission.

#### Example 3

65 The procedure is the same as in Example 2, excepting that there is employed as the 8-hydroxyquinoline color former the compound 5-stearoylamino-3-(8-hydroxy-2-phenylcinchoninoyl)-amino-4-toluenesulfonic acid.

70 Various modifications of the invention will occur to operators in this field, and I accordingly do not intend to be limited in the patent granted except as necessitated by the appended claims.

I claim:

1. The process of producing magenta phenazonium dyestuff images in an exposed silver halide emulsion which comprises developing said

emulsion with a 2,4-diamino aniline developer in the presence of a color former having the following formula:



in which R is an electronegative radical selected from the class consisting of halogen and a mono-nuclear carbocyclic aromatic radical, and R' is a member of the class consisting of hydrogen, carboxy and carbonamido groups containing an alkyl chain of at least 10 carbon atoms.

2. A photographic developer for the production of magenta phenazonium dyestuff images comprising an alkaline solution containing as its essential components a 2,4-diamino aniline developer and as the color former a compound of the following formula:



in which R is an electronegative radical selected from the class consisting of halogen and a mono-nuclear carbocyclic aromatic radical, and R' is a member of the class consisting of hydrogen, carboxy and carbonamido groups containing an alkyl chain of at least 10 carbon atoms.

3. A photographic silver halide emulsion con-

taining as a color former capable of yielding magenta phenazonium dyestuff images a compound of the following formula:



in which R is an electronegative radical selected from the class consisting of halogen and a mono-nuclear carbocyclic aromatic radical, and R' is a member of the class consisting of hydrogen, carboxy and carbonamido groups containing an alkyl chain of at least 10 carbon atoms, at least one of the radicals R and R' containing an alkyl chain of at least 10 carbon atoms.

4. The process as defined in claim 1 wherein the color former is 2-chloro-8-hydroxyquinoline.

5. The photographic developer defined in claim 2 wherein the color former is 2-chloro-8-hydroxyquinoline.

25 6. A photographic silver halide emulsion containing as a color former 5-stearoylamino-3-(8-hydroxy - 2 - phenylcinchoninoyl) -amino-4-toluenesulfonic acid.

ROBERT F. COLES.

#### REFERENCES CITED

The following references are of record in the file of this patent:

#### UNITED STATES PATENTS

35 Number Name Date  
2,306,410 Schinzel Dec. 29, 1942